

W. S. Nelson,

Skating Floor.

No. 86,031.

Patented Jan. 12, 1869.

Fig. 1.



Fig. 2.



Witnesses:

John Becker.  
Wm. A. Morgan.

Inventor:

W. S. Nelson  
Miner L. B.  
Attorney



WILLIAM S. NELSON, OF ST. LOUIS, MISSOURI.

*Letters Patent No. 86,031, dated January 19, 1869.*

IMPROVED SKATING-FLOOR.

The Schedule referred to in these Letters Patent and making part of the same.

*To all whom it may concern:*

Be it known that I, WILLIAM S. NELSON, of St. Louis, in the county of St. Louis, and State of Missouri, have invented a new and improved Skating-Floor; and I do hereby declare that the following is a full, clear, and exact description thereof, which will enable others skilled in the art to make and use the same, reference being had to the accompanying drawings, forming part of this specification, in which—

Figure 1 is a plan view of my invention.

Figure 2 is a section of the same, through the line *x*, *fig. 1.*

Similar letters of reference indicate like parts.

The object of this invention is to provide a surface or floor suitable for skating upon with common runner-skates, and which is designed to be laid in public halls, rinks, parks, and private rooms, for the purpose of skating upon.

It consists, in general terms, in forming a floor of a number of billets or blocks of soft wood fitted together with the grain-ends up, which latter are planed smooth, and treated or prepared, by any suitable materials, to confer on the floor, thus formed, a tough, slippery, and slightly-yielding surface, suitable for skating upon.

In practice, I usually use well-seasoned blocks of white pine or cedar, from two to four inches in length, with their sides and one end planed smoothly.

Before putting these down to form a floor, they are placed, with their planed ends down, in a shallow tank, or vat, containing a strong solution of potash, which soaks into the immersed ends, and gives to them a tough, yielding surface.

After remaining in the potash-solution for a few hours, the blocks are taken out and placed in a second shallow vat containing a melted mixture of tallow and beeswax, and suffered to remain there until the pores of the wood are well filled, which usually requires several hours.

They are then removed, and placed in a warm room until the tallow and beeswax are all dried in.

The blocks, thus prepared, are then laid, with their planed ends up, on a smooth floor of planks, being fastened down in any suitable manner.

In fastening them, I generally bore a central hole into the end of each block, from a third to a quarter of its length, from the upper end, and drive a nail in this hole and through the block into the floor.

The nails are thus countersunk, and the holes are filled up with plugs, which have been previously treated in the same manner as the blocks.

Screws, however, may be used instead of nails, and the blocks may be fastened together and to the floor with cement, of which there are several kinds in use, which would answer the purpose very well.

The blocks being put down, the floor, thus formed by their upper ends, is planed off smooth and evenly, and again treated with two or three coats of the following composition:

One part of beeswax; ten parts of tallow; two parts of pulverized soapstone; one part of Castile soap.

I heat these ingredients together, and apply with a brush while hot. I then rub the surface with hot irons, until the latter composition disappears in the grain of the wood.

I then sift over the surface pulverized soapstone, and rub it in with a block of soft wood, which operation leaves the surface smooth and bright.

The mixture of beeswax and tallow, used after the potash-solution, is in the proportion of one pound of beeswax to nine-tenths of a pound of tallow.

Having thus described my invention,  
I claim as new, and desire to secure by Letters Patent—

A skating-floor, composed of wooden blocks joined together, with the grain-ends upward, and made slippery, in the manner herein shown and described.

WM. S. NELSON.

Witnesses:

DANIEL W. VAN HEUTER,  
H. W. LEFFINGWELL.